# EUROPEAN PATENT SPECIFICATION

(11) **EP 0 159 774 B1**
(45) Date of publication and mention of the grant of the patent: **09.12.1987**
(21) Application number: 85301082.5
(22) Date of filing: 19.02.1985
(51) Int. Cl.: C21D 1/62, C21D 9/573

(54) **Method and apparatus for heat treating steel plates**
Verfahren und Vorrichtung zur Wärmebehandlung von Stahlplatten
Procédé et dispositif pour le traitement thermique de tôles en acier

(30) Priority: 24.02.1984 US 583343
(43) Date of publication of application: 30.10.1985
(73) Proprietor: Van Dorn Company, Cleveland Ohio 44104 (US)
(72) Inventor: Coleman, Vincent R., Aurora Ohio 44202 (US)
(74) Representative: Austin, Hedley William

## Description

The present invention relates to the heat treating of elongated steel members, and, in particular, to a method for continuously leveling and quenching steel plates to provide required flatness without the need of post-quenching leveling and stretching operations.

The invention is particularly directed to the heat treatment of thin steel plates. As is commonly referenced, such plates have a thickness of less than 3/8 inch (.95 cm.) and a width greater than 48 inches (122 cm.) and the invention will be described with particular reference thereto, although it will be hereinafter appreciated that the invention has applicability for widths and thicknesses therebeyond. The invention will also be described with reference to lower carbon alloy steels wherein the rate of quench is very high and residual longitudinal and lateral distortion preceding or following the quenching and/or tempering operations is particularly troublesome. Flatness has reference to the deviation of the top and bottom surface from a horizontal line when the plate is resting on a flat surface. The limit of the deviation is prescribed for varying thicknesses and width. While industry standards, such as ASTM Standard A-G Tables 16-17 is used to prescribe flatness tolerances, more often the customers or heat treaters will have more stringent requirements. All such standards recognize a greater permissible deviation as the plate gauge is reduced below 3/8 inch (9.5 mm). Flatness as used herein thus has prime reference to meeting or exceeding the standards applicable to the final product.

These lower carbon alloy steels, heat treated to improve their physical characteristics, are customarily hot rolled at temperatures between 2100°F-2500°F 1149--1371°C in accordance with known procedures. The rolled plates, as defined from the mill, are reheated to an elevated temperature of 1650°F (898°C) or above to assure complete austenitizing of the steel. Thereafter, the plates are subjected to a quenching operation wherein the plate is rapidly cooled from above its austenitizing temperature to below its Ms .temperature without transformation. Subsequent thereto, the plates undergo a tempering operation whereby the residual stresses are relieved, and hardness and brittleness characteristics are modified and the ductility improved.

While such heat treating procedures readily provide the required physical properties, the ability to provide the required flatness specifications for certain applications is difficult to attain.

Flatness is a particular problem where the steel plate exiting the rolling operation is subject to longitudinal distortion. Therein, the longitudinal dimensions vary from side to side. Thus, if the edges are shorter than the middle portion, the plate will assume a bowed shape. Where the center dimension is shorter than the edge dimensions, the plate will assume a longitudinal lateral waviness. These physical distortions generally arise from processing conditions in the rolling operation. Furthermore, they may only be manifested after reheating in the austenitizing oven and to a lesser extent after tempering. In both instances however, the cause for this distortion has been referenced to the rolling inaccuracies, chemical composition variations and temperature variations, all of which are interrelated.

Due to roll crown or center roller deflection under loading, the plate will often times have a greater thickness at the center than at the edges of the plate. Due to differential cooling, this variation can additionally cause temperature variations across the width and attendent chemical composition variations. Each causes incremental stress variations and yield point variations which are physically manifested during the heating and cooling cycles. Where any of these variations cause uncorrected localized yielding, the ultimate product may be longitudinally and laterally distorted beyond acceptable specification.

Attempts have been made to remedy this post- rolling distortion by leveling intermediate the rolling and the heat treating operations. This has not, however, proven to be a particularly successful technique. While producing apparent leveling, the residual stresses cause the distortions to reappear during reheating. Further, the residual internal stresses may be manifested after heat treatment during shipping and other handling or temperature cycles.

Because of the high yield strength of the end product, generally in excess of 100,000 psi (6894 bar), post heat treating processing through leveling and stretching rolls is also of limited benefit in achieving flatness in the hardened plate.

It has been found that an acceptable flatness can be provided by controlling the conditions during the quenching operation. In my prior patent, United States patent no. 3,604,696, a continuous quenching operation is taught wherein uniformly and rapidly quenching the plate while continuously longitudinally and laterally restraining the plate during the cool down between a series of vertically aligned pressure rolls is effective to provide commercially acceptable flatness. This quench press produces controlled contraction and localized yielding of the plate during quenching thereby eliminating waviness and bowing present in the entering plate. Plates thicker than 3/8 inch (9.525 mm), in particular, can be leveled with such an apparatus, with the flatness being retained or improved, during the subsequent tempering.

Despite this in-treatment leveling, thinner plates oftentimes can not be effectively leveled. As was previously mentioned, post treatment leveling and stretching meets with limited success because of the high yield strength of the hardened plate. Thus, a plate with unacceptable flatness must be recycled through the heat treatment process, or failing that the plate may be designated for off-specification applications or scrap.

### Brief summary of the invention

Accordingly, it is an object of the present invention to provide a method and apparatus for heat treating thin steel plates which produce posttreatment flatness and avoid the need for pre- or post-heat treatment leveling and stretching operations or recycling or scrapping of unacceptable plates.

In accordance with the present invention, thin low carbon steel plates, subject to or prone to lateral and longitudinal distortion, are heated to an elevated temperature above the austenitizing temperature of the steel, preferably in excess of 1650°F (898°C). After sufficient holding time to assure complete austenitizing, the plates, still above the critical temperatures, are rapidly, continuously, reversely flexed without a significant temperature drop. The leveling induces localized yielding and hot working of the plate such that longitudinal and stress equalization of the plate is achieved across its transverse section. This produces a flatness which is within the further leveling capability of the quench press. Immediately after leveling, the plate passes to a quenching operation which rapidly and uniformly cools the plate to below the Ms temperature while laterally and longitudinally restraining the plate such that the plate is cross-sectionally tensioned during the cooling. The tensioned thermal contraction continues the leveling process, further accommodating localized yielding in high stress areas. The entering flatness is maintained or improved and the residual stresses are below the level that would result in further localized yielding as the plate undergoes the subsequent tempering or post treatment handling.

In practicing the aforementioned method, the steel plate, at a temperature above its critical temperature, is longitudinally fed through a series of alternating decreasingly vertically offset rollers at a high rate of speed and without an appreciable temperature drop. The initial vertical offset is sufficient to cause localized yielding of the shorter longitudinal section lengths where the yield strength at this temperature is only 2-3% of that of the finished product. The subsequent offsets are progressively reduced to hot flex the plate for stress equalization. The preliminarily flattened plate is then fed between a series of vertically aligned cylindrical quench rolls. Quenching jets between the rolls uniformly supply coolant at a rate which rapidly and uniformly lowers the temperature of the plate through the martinsite range without transformation. Successive pairs of the rollers are effective to locally tension the plate during the quenching. This accommodates further localized thermal contraction and yielding as required while maintaining plate flatness. At the end of the quenching operations, the internal stresses are below a level which will cause yielding of the plate during the temperature excursion of the subsequent tempering operation.

In this manner, the plate exiting the quenching press will have achieved a flatness equal to or greater than the flatness provided in the leveling operation and a flatness which is not negatived during the heating and cooling of tempering.

It will become apparent that the present invention offers a substantial advance in providing heat treatment leveling of steel plates wherein sequential controlled yielding and stress equalization of the plate during the heating and cooling cycles is used to achieve and maintain a flattened condition thereby avoiding the need for subsequent stretching operations and limiting material subject to recycling or scrapping.

### Brief description of the drawing

These and other advantages of the present invention become apparent to one skilled in the art upon consideration of the following specification with reference to the accompanying drawings in which:
Figure 1 is a side elevational view of a heat treating unit made in accordance with the present invention;
Figure 2 is an enlarged elevational view showing the leveling assembly of the heat treating unit of Figure 1;
Figure 3 is a partially broken end view taken along line 3-3 in Figure 1;
Figure 4 is a partially broken top view of the heat treating unit shown in Figure 1;
Figure 5 is a schematic elevational view of the heat treating unit illustrating the principles of the present invention; and,
Figure 6 is a schematic elevational view of the drive trains for the leveling and quenching assemblies.

### Detailed description of the invention

Referring to the drawings for purposes of illustrating the preferred embodiment of the invention only and not for the purpose of limiting the same, there is shown in Figure 1 a heat treating unit 10 for continuously leveling and quenching thin low carbon steel plates 12. The plates 12 travel horizontally from an austenitizing furnace 14 through the unit 10 into a tempering furnace 16.

As is conventional in heat treating such steels, the plate 12 is heated in the austenitizing furnace 14 to a temperature above its critical temperature for a sufficient time to assure complete austenitizing of the steel. Generally the furnace temperature is in excess of 1650°F (898°C), preferably over 1700°F (927°C). The plate 12 is then rapidly and uniformly cooled in a quenching operation through the Ms temperature and through the Mf temperature to transform the austenite to martensite. The quenched plate is then reheated to an elevated temperature in the tempering furnace 16 for improving the strength characteristic. The temperatures and times are dependent in a conventional manner upon the composition of the alloy and the ultimate properties desired.

The present invention is particularly suited for thin steel plates having a thickness of less than around 3/8 inch and having a width in excess of 14 inches. Such plates, because of the preceding hot rolling, temperature variations and chemical composition variations, are particularly prone to distortion exiting the austenitizing oven, and to certain extents, subsequent to the tempering operation. However, it will be apparent that the benefits of the invention apply as well for plates of greater thicknesses and lesser widths.

The aforementioned distortions are physically characterized by variations in the longitudinal edge length compared to the length of the center portion. Accordingly, where the length of the longitudinal edge is greater than the longitudinal length of the center section, the edge will assume a wavy appearance. Where the longitudinal edges are shorter than the center section, the plate will assume a bowed or fluted shape. This can cause a horizontal deviation of 12 inches or more. By use of the subject heat treating apparatus, such entering distortions are removed and the tendency to form such distortions in the final product are eliminated.

More particularly, the heat treating unit 10 comprises a frame assembly 20 having downwardly depending legs 21 appropriately connected to a foundation 22 surrounding a quench basin 23. The frame assembly 20 includes a fixed lower framework 24 and an upper framework 26 supported on end sections 28 disposed at either end of the frame assembly 20 and vertically movable with respect to the lower frame member.

Disposed interior of the frameworks 24 and 26 are a leveling assembly 30 adjacent the entry end of the heat treating unit 10 and a quenching assembly 32 adjacent the exit end of the unit 10. The overall size of the unit will be determined by the size capability of the unit for treating an array of plate sizes and thickness. However, a unit for heat treating plates of up to 108 inches (2743 mm) wide, in thicknesses to below 1/4 inch (6,35 mm), to conventional hardnesses would be in the order of 30 feet (9.14 m) long by 8 feet (2.438 m) high by 10 feet (3.048 m) wide.

Three pinch roll assemblies 34 are longitudinally disposed along the frame assembly 20, one being positioned at the entry end in advance of the leveling assembly 30, one positioned intermediate the leveling assembly 30 and quenching assembly 32, and one positioned after the quenching assembly 32. The opposed nips of the upper and lower roller sets of the leveling assembly 30, the quenching assembly 32 and the pinch roll assemblies 34 define a horizontal path 36 through which the plate 11 longitudinally travels during the leveling and quenching operations.

The pinch roller assemblies 34 comprise a lower roll 38 and an upper roll 39 and are operative to longitudinally feed the plate through the unit. The pinch rolls may be solid or hollow cylinders with a diameter of about 10" (25,4 cm). The lower rolls 38 are fixedly connected to and rotatably supported by bearing chocks 40 on the lower framework 24. The upper rolls 39 are fixedly connected to and rotatably supported by bearing chocks 41 on the upper framework 26. The axes of rotation of the lower roll 38 and the upper roll 39 are transverse to the longitudinal path 36 and lie in a common vertical plane. The nips of the lower rollers 38 lie in a common lower horizontal plane. The nips of the upper rollers 40 lie in a common upper horizontal plane. In operation, the lower rolls compressively and frictionally engage the bottom surface of the plate and the upper rolls compressively and frictionally engage the top surface of the plate during movement along the path 36 through the leveling and quenching operations as loaded by the upper framework 36.

The feed rate and loading are predetermined by the size, thickness, composition and desired properties for the plates being treated.

Referring to Figure 2, the leveling assembly 30 includes alternating upper and lower rolls. More particularly, six equally longitudinally spaced lower rolls 42 are rotatably supported on a base assembly 43 fixedly connected to the lower framework 24. The lower rolls 42 have axes of rotation transverse to the path 36. The nips of the individual lower rolls 42 lie in a horizontal plane coextensive with the plane defined by the nips of the lower pinch roll 38. The lower rolls 42 have their outer contours locally engaging the bottom surface of the plate 12. Five equally longitudinally spaced upper rolls 44, mounted on a upper base assembly 46 are disposed vertically intermediate the lower rolls 42. The axes of rotation of the upper rolls 44 are transverse to the path 36 and lie in a common pivotally adjustable plane.

Similar to the rolls of the quenching assembly which are shown in Figure 3, the leveling rolls have a solid cross-section and a roll diameter of about 6 inches. The individual rolls are centrally longitudinally divided into two rolling sections and are rotatably supported at their ends and middle by bearing chocks.

The base assembly 46 is pivotally connected at an inner end to the upper framework 26 by pin connection 48. The outer end of the assembly 46 is operatively connected to a drive unit 50 mounted on the upper framework 26. The drive unit 50 is manually adjustable by drive wheel 52 to raise or lower shaft 53 to pivot the rolls 44 about the pin connection 48 thereby progressively raising or lowering the upper rolls 44 between the lower rolls 42. The movement of the upper rolls 44 is visually determined by a pivoting indicator arm 51 and scale 55. Accordingly, an entering plate passing between the leveling rolls will be alternatingly downwardly and upwardly flexed by the leveling assembly with progressively lesser flexing toward the inner end of the assembly. Should uniform progressive flexing of the plate be desired, the rolls 44 can be vertically adjustable as a unit with respect to the upper framework and lower rolls. However, the progressive roller arrangement is effective in initially removing the longitudinal distortion with the subsequent leveling being of a less severe nature to progressively flex and hot work the plate to equalize the internal stresses.

The leveling assembly has been described with eleven rolls. However, it will be appreciated that any number greater than three can be utilized depending on the required processing capabilities of the unit.

The quenching assembly comprises lower and upper roll assemblies 54 and 56 respectively. The lower roller assembly 54 is fixedly connected to the lower framework 24. The upper assembly 56 is fixedly connected to the upper framework 26. The assemblies 54 and 56 carry a plurality of vertically opposed, equally longitudinally spaced lower rolls 58 and upper rolls 60. The lower rollers 58 have axes of rotation transverse to the path 36 with the nips thereof lying in a horizontal plane coextensive with the nips of the lower pinch rolls 38. The axes of rotation of the upper rolls 60 lie in a common vertical plane with the opposed rolls 58 transverse to the path 36 in a horizontal plane coextensive with the nips of the upper pinch rolls.

Referring to Figure 3, the individual rolls are six inches in diameter and are longitudinally divided in two roller sections. The rolls are rotatably supported by bearing chocks at their ends and middle sections to limit center deflection under rolling conditions. It will be appreciated however, that a continuous contour could be provided by the use of backup rollers. The rolls and back up rollers may be provided with internal cooling for enhancing the uniformity of cooling during quenching.

In operation, the lower rolls 58 compressively and frictionally engage the bottom surface of a plate. The upper rolls 60 compressively and frictionally engage the top surface of the plate. Either or both of the roll assemblies may be spring biased toward the other so as to establish varying levels of compressive engagement with the plate.

Quenching jets 62 are disposed on either side of the plate and longitudinally between successive rolls throughout the quenching assembly. The jets 62 are respectively fluidly connected by pipes 63 to a main supply conduit 64 extending along the length of the upper frame 26. The flow rates of the individual jets 62 are controlled by valves 66. As previously mentioned, the individual rolls are preferably internally cooled as well. The general fluid interconnections are operative to provide uniform but varying rates of cooling of the plate in a number of longitudinal zones as it traverses the quenching assembly, in a manner consistent with the method and apparatus set forth in the aforementioned United States patent no. 3,604,696.

The drive means for raising and lowering the upper framework 26 with respect to the lower framework 24, includes right angle drive units 70 disposed in pairs on the opposed end sections of the framework 26. The units 70 are operatively interconnected by drive shafts 72. The units 70 carry input sprockets which are connected by a continuous roller chain to sprockets mounted on drives 74. The input of the drives 74 are interconnected by drive shafts 76 to a centrally located duel output drive unit 78. The input of the unit 78 is operatively connected to a motor and speed reducer assembly, not shown. Accordingly, upon energization of the motor and speed reducer assembly, the drive means are effective to simultaneously drive the units 70 to guide the framework vertically and uniformly along threaded posts supported on the top of the end sections 28. The overall weight of the upper framework establishes the loading between the pinch rollers, the leveling rolls and the quench rolls with respect to the plate 12. The drive means are vertically adjusted for accommodating plates of varying thicknesses.

Referring to Figure 6, the drive trains for roll to roll driving are schematically shown. More particularly, the first two upper pinch rolls 39 and the upper leveling rolls 44 are drivingly interconnected as a set by a roller chain and sprocket drive 90. Sprockets are mounted on the outer ends of individual rolls at both sides of the upper frame members. The first two lower pinch rolls 38 and the lower rolls 42 of the leveling assembly 30 are similarly interconnected by a second chain and sprocket drive 92. The sprockets are mounted on the outer ends of the associated roller on both sides of the upper frame. Each drive 90 and 92 includes idler and adjustment sprockets 94 and 96 respectively. Secondary sprockets of the inner pinch rolls are interconnected by a roller chain 99. One of these sprockets is drivingly connected to an electric motor and speed reducer assembly 100. Accordingly, all of the interconnected rollers are driven at the same peripheral speed for advancing the plate through the leveling unit. Because of the common peripheral speed through the leveling unit, the plate is not fed under tension. However, if desired, tensioning may be provided through sprocket changes or the like.

The lower rolls of the quenching assembly and the remote pinch roll assembly 34 are drivingly interconnected by a chain and sprocket drive 102. The upper rolls are idler rolls.

The sprockets are mounted on the outer ends of the rolls at the sides of the lower framework 24. The drive 102 includes idler and adjustment sprockets 104.

The sprockets of the intermediate pinch roll is interconnected to the sprocket of the inner quench roll by drive chain 106. The drives are effective to rotate the lower quench rollers, the leveling rolls and the pinch rolls at the same peripheral speed. If desired, the peripheral speed in the quenching assembly may vary with respect to that of the leveling assembly by providing independent drives so as to directly tension the plate during the contraction of the plate in the quenching operation. It should be further apparent that the intermediate pinch roll assembly may also constitute a driven element in the quench drive transmission with the relative speed being adjusted to provide the same overall effect.

### Operation of the preferred embodiment

Steel plates as received from the rolling mill are reheated in the austenitizing furnace 14 to an

elevated temperature in excess of the critical temperature of the alloy. The actual temperature is such that all carbides are in solution to take full advantage of the hardenability of the particular steel involved. In general, this temperature will be 1650° (898°C) or higher, preferably around 1700°F (927°C). As delivered, the steel plates may have initial longitudinal distortion, or as commonly is the case upon reheating in the austenitizing furnace 14, residual stresses due to variations in the rolling procedure and chemical compositions may cause the generally flat as-received plate to assume such distorted condition. Further, such plate may be prone post-heat treatment distortion following the tempering or subsequent handling.

To ready the apparatus 10 forthe heat treatment of a particular width and thickness of plate, the upper framework 26 is adjusted by the quench press lift drive to receive the plate with the upper framework exerting a compressive loading at the nips of the pinch roller assemblies and the rollers of the quenching assembly 32. This loading will be sufficient to maintain the desired loading and feeding as a plate travels through the assembly while locally and laterally restraining the moving plate. Depending on the anticipated or historical distortion of the plates, the leveling assembly 30 is adjusted by means of drive 50 to pivot the upper leveling rolls 44 with respect to the lower rolls 42 provide the necessary vertical offsets and flexing to remove the longitudinal distortions and equalize the stresses.

The feed rate provided by the pinch rolls is at a predetermined rate, dependent upon the temperature, the alloy, its thickness and other factors.

Referring to Figure 5, the plate passes through the leveling assembly and is alternately downwardly and upwardly flexed along the contours of the leveling rolls exiting the final lower roll in a substantially leveled condition before entering the intermediate pinch rollers. This pass lengthens the shorter longitudinal sections of the plate, which have contributed the waviness or fluting, beyond their elastic limit thereby locally lengthening and equalizing the incremental lengths. Inasmuch as the pinch rolls of the first two sets are driven at a common peripheral speed, the sheet is not subjected to any tensile loading within the leveler, the localized leveling through yielding merely establishing length uniformity and stress equalizations through the reverse flexing operation. Should it be desired to establish tensile loading on the sheet during the leveling operation, the same may be effected through conventional means. For instance, a change in sprocket gearing or coupling. the intermediate roller to the drive chain of the quench assembly could be used to achieve a differential speed with respect to the peripheral drive speed in the leveler rolls.

It is preferred to locate the unit as closely as possible to the austenitizing furnace so as to minimize any cool down of the plate prior to the quenching operation. This is particularly important for the thin plates of the present invention. This is further minimized by driving the plate through the unit at a high rate of speed in the order of 20 to 200 feet (6.09 to 60.96 m) per minute such that they pass through the leveling operation without any substantial reduction in the temperature and arrive at the quenching operation at the aforementioned figure of around 1650°F (898°C) or above. The leveled plates then pass through the longitudinal series of quenching rollers under lateral and longitudinal tensioning and outwardly of the unit from the final pinch rollers into the tempering furnace 16.

During the quenching operation, the flow rates through the quench jets are adjusted to provide varying quenching zones such that the plates pass from the austenitizing temperature through the martinsite transformation temperature range at a rate rapid enough to prevent any transformation, and to provide substantial uniformity and hardening throughoutthe plate. Depending on the thickness of the plate and the alloy composition, the feed rate and quenching adjustments are appropriately controlled.

The lateral and longitudinal constraints provided by the quenching rollers, tensions the plate during thermal contraction.

This lateral and longitudinal incremental and overall tensioning thus maintains the entering flatness from the leveling assembly and the thermal contraction is effective to cause any remaining or newly developed localized deviations to assume planarity during quenching. This also is effective to accommodate localized yielding, to the extent the yield strength is exceeded at the prevailing temperature, and further stress equalization. The residual stresses in the plate upon relaxation following the quenching operation will be below the yield point of the material during the thermal cycle of the tempering operations. As such, the plate retains its flatness throughout the tempering cycle. Further downstream operations for leveling and stretching are not required for the finished sheet. This is particularly advantageous inasmuch as the yield strength of the hardened and tempered steel is around 80,000-100,000 psi (5516-6895 bar) or above where it has been found to be virtually impossible to remove residual distortions. Further, the hardened plate undergoing such operations is subject to unacceptable surface cracking. The flatness achieved in the subject apparatus also substantially reduces and eliminates the need for recycling plates through the heat-treated cycle which do not meet flatness specifications or those the designated for off-specification application or scrap if recycling does not produce the desired flatness.

The invention has been above described with reference to the preferred embodiment. Obviously, modifications and alterations will occur to those skilled in the art upon reading of this detailed description. It is my intention to include all such modifications and alterations insofar as they come within the scope of the appended claims.

## Claims

1. An apparatus for the leveling and heat treating of steel plates comprising:
platform means;
first frame means fixedly connected to the platform means;
second frame means carried by the platform means for vertical movement with respect to the first frame means, said first frame means and said second frame means defining therebetween a longitudinal path for movement of the steel plates;
first drive means for adjustably moving the first frame means with respect to second frame means;
first leveling rolls fixedly rotatably carried by one of the frame means, said first leveling rollers being arranged in a longitudinal series adjacent the entry end of the longitudinal path and having axes of rotation lying transverse to the longitudinal path with the nips thereof lying in a common horizontal plane;
second leveling rolls adjustably carried by other frame means, and arranged in a longitudinal series adjacent the entry end of the longitudinal path and having axes of rotation lying transverse to the longitudinal path and longitudinally spaced intermediate to the axes of the first leveling roller means;
second drive means for moving the second leveling rollers with respect to the first leveling rolls to at least a position vertically intermediate the horizontal plane of the first leveling rollers and the axes thereof to thereby establish a reversely bending pathway for a steel plate trans- versing the longitudinal path to reversely bend to plate beyond the localized yield point to thereby establish a substantially transversely uniform lonqitudinal length for the plate;
third drive means for rotating the leveling roll means at a common peripheral speed;
a first set of quench rolls arranged in a longitudinal series and carried by the first frame means adjacent the exit end of the longitudinal path, said first quench roll means having axes of rotation transverse to the longitudinal path and with the nips lying in a common horizontal plane;
a second set of quench rolls arranged in a longitudinal series carried by the second frame means adjacent the end of the longitudinal path, said second sets quench rollers having axes of rotation transverse to the longitudinal path with individual axes of rotation being in a common vertical plane with an axis of an opposed roller of said first set of quench rolls and with the outer nips thereof adapted to compressively engage the other surface of the plate, the arrangement being such that the nips of the rolls are adapted to longitudinally and laterally restrain localized portions of the plate during movement of the plate along the path;
fourth drive means for rotating one set of quench rolls at a peripheral speed independent of the third drive means whereby the third and fourth drive means are operative to longitudinally drive the plate along the rolls; and,
quench means disposed between the quench roller means for uniformly quenching a plate moving along the path.

2. The apparatus as recited in claim 1 wherein said second leveling rolls are adjustably pivotally carried by said other frame means and adapted to provide decreasing reverse bending of a plate travelling between said first leveling rolls and said second leveling rolls toward said quench rolls.

3. The apparatus as recited in claim 1 wherein pinch roll means carried by the frame means are additionally operative to longitudinally feed the plate along the longitudinal path as driven by said third drive means and said fourth drive means.

4. The apparatus as recited in claim 3 wherein said pinch roll means include a first roll set of vertically aligned rolls respectively carried by said frame means disposed at the entry end of the leveling rolls, a second set of vertically aligned rolls respectively carried by said frame means intermediate said leveling rolls and said quench rolls, and a third set of vertically aligned pinch rolls respectively carried by said frame means disposed at the exit end of said quench rolls.

5. The apparatus as recited in claim 4 wherein said first set of pinch rolls and said second set of pinch rolls are rotated at a common peripheral speed with the leveling rolls by said third drive means so as to longitudinally feed the plate through the leveling rolls without longitudinal tensioning of the plate.

6. The apparatus as recited in claim 5 wherein said third set of pinch rolls and one set of quench rolls are rotated at a common peripheral speed by said fourth drive means.

7. The apparatus as recited in claim 6 wherein said third drive means and said fourth drive means are drivingly connected to rotate the associated rolls at the same peripheral speeds.

8. A method of heat treating steel plates subject to longitudinal distortion comprising the steps of:
passing the plate along a reversely bending path at a temperature above the critical temperature of the steel to longitudinally stress the plate beyond the yield strength thereof at said temperature above said critical temperature to establish substantial uniformity of longitudinal length throughout said plate, thereby removing said longitudinal distortion; and,
passing the plate along a quenching path while rapidly uniformly cooling the plate from the above the critical temperature to below the martensite temperature thereof while incrementally longitudinally and laterally restraining the plate to thereby retain the uniformity of longitudinal length.

9. The method as recited in claim 8 wherein said temperature is around 1650°F (898,9°C) or above.

10. The method as recited in claim 9 wherein the plate exits said reversely bending without appreciable temperature drop and at a temperature above around 1650°F (898,9°C) or above.

11. The method as recited in claim 10 wherein said reversely bending path has progressively decreasing curvature to provide hot working of the plate and stress equalization therewithin subsequent to establishing said substantial uniformity of longitudinal length.

12. The method as recited in claim 11 wherein the plate passes along said reversely bending path without longitudinal tensioning.

13. The method as recited in claim 8 wherein the plate is longitudinally stressed in said reversely bending path in the range of 2,000 to 3,000 psi (137,9-206,8 bar).

14. The method as recited in claim 13 comprising the further step of holding the plate in an austenitizing oven at a temperature above said critical temperature and immediately passing the plate through said reversely bending path without an appreciable temperature drop.

15. The method as recited in claim 14 wherein said plate is passed along said paths at a speed in the range of 20 to 200 feet per minute.

16. The method as recited in claim 8 wherein the stresses in the plate following quenching are equalized sufficiently to prevent subsequent longitudinal distortion in a tempering operation.

17. A method for leveling steel plates subject to transverse variations in longitudinal length comprising the step of:
progressively reversely flexing the plate at a temperature above the austenite temperature of the steel at a loading in the range around 2,000 to 3,000 psi (137,9-206,8 bar) sufficient to substantially remove the transverse variations in longitudinal length.

18. The method as recited in claim 17 including progressively decreasing the flexing of the plate to promote stress equalization within the plate.

## Patentansprüche

1. Vorrichtung zum Richten und zur Wärmebehandlung von Stahlplatten, die enthält:
Plattenformmittel;
erste Rahmenmittel, die fest mit dem Plattformmittel verbunden sind;
zweite Rahmenmittel, die gegenüber den ersten Rahmenmitteln vertikal beweglich von dem Plattformmittel getragen werden, wobei die ersten Rahmenmittel und die zweiten Rahmenmittel einen Längsweg für die Bewegung der Stahlplatten zwischen sich bilden;
erste Antriebsmittel zum einstellbaren Bewegen der ersten Rahmenmittel gegenüber den zweiten Rahmenmitteln;
erste Richtwalzen, die von einem der Rahmenmittel fest angebracht drehbar getragen werden, wobei die ersten Richtwalzen in einer längsverlaufenden Reihe an das Eintrittsende des Längsweges anschließend angeordnet sind und Drehachsen haben, die quer zu dem Längsweg liegen und deren Berührungslinien in einer gemeinsamen Horizontalebene liegen;
zweite Richtwalzen, die einstellbar von den anderen Rahmenmitteln getragen werden und in einer längsverlaufenden Reihe neben dem Eintrittsende des Längsweges angeordnet sind und Drehachsen haben, die quer zu dem Längsweg liegen und die in Längsrichtung im Abstand voneinander zwischen den Achsen der ersten Richtwalzenmittel sich befinden;
zweite Antriebsmittel zum Bewegen der zweiten Richtwalzen gegenüber den ersten Richtwalzen mindestens bis zu einer Stellung, die sich vertikal zwischen der Horizontalebene der ersten Richtwalzen und deren Achsen befindet, um hierdurch für eine den Längsweg durchlaufende Stahlplatte einen Rückbiegeweg zu schaffen, auf dem die Platte jenseits der lokalisierten unteren Streckgrenze rückgebogen wird, um hierdurch eine über die Breite im wesentlichen gleichförmige Länge der Platte zu erreichen;
dritte Antriebsmittel zum Drehen der Richtwalzenmittel mit einer gemeinsamen Umfangsgeschwindigkeit;
einen ersten Satz Abschreckwalzen, die in einer in Längsrichtung verlaufenden Reihe angeordnet sind und von den ersten Rahmenmitteln anschließend an das Ausgangsende des Längsweges getragen werden, wobei die genannten ersten Abschreckwalzenmittel Drehachsen haben, die quer zu dem Längsweg verlaufen und wobei die Berührungslinien der Walzen in einer gemeinsamen, horizontalen Ebene liegen;
einen zweiten Satz Abschreckwalzen, die in einer längs verlaufenden Reihe angeordnet sind und von den zweiten Rahmenmitteln an das Ende des Längsweges anschließend getragen werden, wobei der genannte zweite Satz Abschreckwalzen Drehachsen hat, die quer zum Längsweg verlaufen und wobei die einzelnen Drehachsen sich mit je einer Achse einer gegenüberliegenden Walze des genannten ersten Abschreckwalzensatzes in einer gemeinsamen, vertikalen Ebene befinden und wobei die äußeren Berührungslinien dieser Walzen dazu geeignet sind, drükkend auf die andere Oberfläche der Platte einzuwirken und wobei die Anordnung so getroffen ist, daß die Berührungslinien der Walzen örtlich begrenzte Teile der Platte während ihrer Bewegung längs des Weges längs und quer zurückhalten können;
vierte Antriebsmittel zum Drehen eines Abschreckwalzensatzes mit einer von der Umfangsgeschwindigkeit der dritten Antriebsmittel unabhängigen Umfangsgeschwindigkeit, wobei die dritten und vierten Antriebsmittel wirksam sind, um die Platte in Längsrichtung längs der Walzen zu treiben;
Abschreckmittel, die zwischen den Abschreckwalzenmitteln angeordnet sind, zum gleichförmigen Abschrecken einer Platte, die sich längs des Weges bewegt.

2. Vorrichtung nach Anspruch 1, bei der die genannten zweiten Richtwalzen von dem genannten anderen Rahmenmittel einstellbar schwenkbar getragen werden und geeignet sind, eine abnehmende Rückbiegung der zwischen den ersten Richtwalzen und den zweiten Richtwalzen zu den Abschreckwalzen durchlaufenden Platte vorzusehen.

3. Vorrichtung nach Anspruch 1, wobei von dem Rahmenmittel getragene Klemmwalzenmittel zusätzlich wirksam sind, um die Platte in Längsrichtung längs des Längsweges zu befördern, während sie von dem genannten dritten Antriebsmittel und dem genannten vierten Antriebsmittel angetrieben werden.

4. Vorrichtung nach Anspruch 3, wobei die genannten Klemmwalzenmittel einen ersten Walzensatz von vertikal in einer Linie übereinander angeordneten Walzen aufweisen, die von den genannten Rahmenmitteln getragen werden und am Eingangsende der Richtwalzen angeordnet sind, einen zweiten Satz von vertikal in einer Linie übereinander angeordneten Walzen, die von den genannten Rahmenmitteln getragen werden und zwischen den genannten Richtwalzen und den genannten Abschreckwalzen angeordnet sind, und einen dritten Satz von vertikal übereinander angeordneten Klemmwalzen, die von den genannten Rahmenmitteln getragen werden und am Ausgangsende der genannten Abschreckwalzen angeordnet sind.

5. Vorrichtung nach Anspruch 4, wobei der genannte erste Satz Klemmwalzen und der genannte zweite Satz Klemmwalzen von den genannten dritten Antriebsmitteln mit der gleichen Umfangsgeschwindigkeit gedreht werden wie die Richtwalzen, so daß die Platte in Längsrichtung durch die Richtwalzen gefördert wird ohne daß die Platte einer Längsdehnung unterworfen wird.

6. Vorrichtung nach Anspruch 5, wobei der genannte dritte Satz Klemmwalzen und ein Satz Abschreckwalzen von dem genannten vierten Antriebsmittel mit einer gemeinsamen Umfangsgeschwindigkeit gedreht werden.

7. Vorrichtung nach Anspruch 6, wobei das genannte dritte Antriebsmittel und das genannte vierte Antriebsmittel antriebsverbunden sind, um die zugeordneten Walzen mit den gleichen Umfangsgeschwindigkeiten zu drehen.

8. Verfahren zur Wärmebehandlung von Stahlplatten, die einer Längsverwerfung ausgesetzt sind, das folgende Verfahrensschritte enthält:
Führen der Platte längs eines Rückbiegeweges bei einer oberhalb der kritischen Temperatur des Stahles liegenden Temperatur, um die Platte jenseits der Streckgrenze bei der genannten Temperatur oberhalb der genannten kritischen Temperatur in Längsrichtung zu dehnen und im wesentlichen Gleichförmigkeit der Längenausdehnung überall in der Platte zu erreichen und hierdurch die genannte Längsverwerfung zu beseitigen;
Führen der Platte längs eines Abschreckweges, während die Platte schnell und gleichförmig von oberhalb ihrer kritischen Temperatur auf unterhalb ihrer Martensittemperatur abgekühlt wird, während die Platte zusätzlich in Längs- und Querrichtung zurückgehalten wird, um hierdurch die Gleichförmigkeit der Länge beizubehalten.

9. Verfahren nach Anspruch 8, wobei die genannte Temperatur bei 1650°F (898,9°C) oder darüber liegt.

10. Verfahren nach Anspruch 9, wobei die Platte die genannte Rückbiegung ohne nennenswerten Temperaturabfall und bei einer Temperatur von oberhalb etwa 1650°F (898,9°C) oder darüber verläßt.

11. Verfahren nach Anspruch 10, wobei der genannte Rückbiegeweg eine fortschreitend abnehmende Krümmung hat, um eine Warmformgebung der Platte und einen Spannungsausgleich in dieser im Anschluß an das Herstellen der genannten, annähernden Gleichförmigkeit in der Länge zu erreichen.

12. Verfahren nach Anspruch 11, wobei die Platte den genannten Rückbiegeweg ohne Längsspannen durchläuft.

13. Verfahren nach Anspruch 8, wobei die Platte in dem genannten Rückbiegeweg in der Größenordnung von 2000 bis 3000 PSI (137,9 bis 206,8 bar) in Längsrichtung gespannt wird.

14. Verfahren nach Anspruch 13, welches den weiteren Schritt enthält, bei dem die Platte in einem Austenitisierofen bei einer oberhalb der genannten kritischen Temperatur liegenden Temperatur gehalten und ohne nennenswerten Temperaturabfall unmittelbar durch den genannten Rückbiegeweg geführt wird.

15. Verfahren nach Anspruch 14, wobei die genannte Platte mit einer Geschwindigkeit in der Größenordnung von 20 bis 200 Fuß/Minute längs der genannten Wege geführt wird.

16. Verfahren nach Anspruch 8, wobei die Spannungen in der Platte nach dem Abschrecken genügend ausgeglichen werden, um eine nachfolgende Längsverwerfung bei einer Anlaßbehandlung zu verhüten.

17. Verfahren zum Ebnen von Stahlplatten, die Querveränderungen in ihrer längsverlaufenden Länge unterworfen sind, das folgenden Verfahrensschritt enthält:
Fortschreitende Rückbiegung der Platte bei einer Temperatur, die oberhalb der Austenittemperatur des Stahles liegt, bei einer Beanspruchung in der Größenordnung von etwa 2000 bis 3000 PSI (137,9 bis 206,8 bar) die ausreichend ist, um die Querveränderungen in der längsverlaufenden Länge im wesentlichen zu beseitigen.

18. Verfahren nach Anspruch 17 einschließlich fortschreitendes Verringern der Biegung der Platte, um den Spannungsausgleich in der Platte zu fördern.

## Revendications

1. Appareil pour le dressage et le traitement thermique de tôles d'acier comprenant:
une plate-forme;
un premier châssis relié fixement à la plate-forme;
un second châssis porté par la plate-forme afin de pouvoir se déplacer verticalement par rapport au premier châssis, ledit premier châssis et ledit second châssis définissant entre eux un chemin longitudinal pour le mouvement des tôles d'acier;
des premiers moyens d'entraînement destinés à déplacer de façon réglable le premier châssis par rapport au second châssis;
des premiers cylindres de dressage portés en position fixe et de façon à pouvoir tourner par l'un des châssis, lesdits premiers cylindres de dressage étant disposés en une série longitudinale adjacente à l'extrémité d'entrée du chemin longitudinal et leurs axes de rotation s'étendant transversalement au chemin longitudinal, leurs zones de serrage s'étendant dans un plan horizontal commun;
des seconds cylindres de dressage portés de façon réglable par l'autre châssis et agencés en une série longitudinale à proximité immédiate de l'extrémité d'entrée du chemin longitudinal, leurs axes de rotation s'étendant transversalement au chemin longitudinal et étant espacés longitudinalement entre les axes des premiers cylindres de dressage;
des deuxièmes moyens d'entraînement destinés à déplacer les seconds cylindres de dressage par rapport aux premiers cylindres de dressage vers au moins une position située verticalement entre le plan horizontal des premiers cylindres de dressage et leurs axes afin d'établir ainsi un trajet de cintrage alterné pour une tôle d'acier parcourant le chemin longitudinal de façon à cintrer de manière alternée la tôle au-delà de la limite apparente localisée d'élasticité pour donner ainsi une longueur longitudinale sensiblement transversalement uniforme à la tôle;
des troisièmes moyens d'entraînement destinés à faire tourner les cylindres de dressage à une vitesse périphérique commune;
un premier jeu de cylindres de trempe agencés enune série longitudinale et portés par le premier châssis à proximité immédiate de l'extrémité de sortie du chemin longitudinal, lesdits premiers cylindres de trempe ayant des axes de rotation transversaux au chemin longitudinal et leurs zones de serrage s'étendant dans un plan horizontal commun;
un second jeu de cylindres de trempe agencés en une série longitudinale portés par le second châssis à proximité immédiate de l'extrémité du chemin longitudinal, les cylindres de trempe dudit second jeu ayant des axes de rotation transversaux au chemin longitudinal, les axes individuels de rotation étant situés dans un plan vertical commun, avec un axe d'un cylindre opposé dudit premier jeu de cylindres de trempe et leurs zones de serrage extérieures conçues pour s'appliquer par compression contre l'autre surface de la tôle, l'agencement étant tel que les zones de serrage des cylindres sont conçues pour retenir longitudinalement et latéralement des parties localisées de la tôle durant le mouvement de la tôle le long du chemin;
des quatrièmes moyens d'entraînement destinés à faire tourner un jeu de cylindres de trempe à une vitesse périphérique indépendante des troisièmes moyens d'entraînement afin que les troisièmes et quatrièmes moyens d'entraînement aient pour effet d'entraîner longitudinalement la tôle le long des cylindres; et
des moyens de trempe disposés entre les cylindres de tempe afin de tremper uniformément une plaque se déplaçant le long du chemin.

2. Appareil selon la revendication 1, dans lequel lesdits seconds cylindres de dressage sont portés de façon pivotante et réglable par ledit autre châssis et sont conçus pour produire un cintrage alterné décroissant d'une tôle avançant entre lesdits premiers cylindres de dressage et lesdits seconds cylindres de dressage vers lesdits cylindres de trempe.

3. Appareil selon la revendication 1, dans lequel des cylindres entraîneurs portés par le châssis sont en outre mis en oeuvre pour faire avancer longitudinalement la tôle le long du chemin longitudinal sous l'action desdits troisièmes moyens d'entraînement et desdits quatrièmes moyens d'entraînement.

4. Appareil selon la revendication 3, dans lequel lesdits cylindres entraîneurs comprennent un premier jeu de cylindres alignés verticalement, portés respectivement par ledit châssis et disposés à l'extrémité d'entrée des cylindres de dressage, un deuxième jeu de cylindres alignés verticalement, portés respectivement par ledit châssis entre lesdits cylindres de dressage et lesdits cylindres de trempe, et un troisième jeu de cylindres entraîneurs alignés verticalement, portés respectivement par ledit châssis et disposés à l'extrémité de sortie desdits cylindres de trempe.

5. Appareil selon la revendication 4, dans lequel ledit premier jeu de cylindres entraîneurs et ledit deuxième jeu de cylindres entraîneurs sont mis en rotation à une vitesse périphérique commune avec les cylindres de dressage par lesdits troisièmes moyens d'entraînement afin de faire avancer longitudinalement la tôle entre les cylindres de dressage sans appliquer une tension longitudinale à la tôle.

6. Appareil selon la revendication 5, dans lequel ledit troisième jeu de cylindres entraîneurs et un jeu de cylindres de trempe sont mis en rotation à une vitesse périphérique commune par lesdits quatrièmes moyens d'entraînement.

7. Appareil selon la revendication 6, dans lequel lesdits troisièmes moyens d'entraînement et lesdits quatrièmes moyens d'entraînement sont reliés en prise afin de faire tourner les cylindres associés aux mêmes vitesses périphériques.

8. Procédé de traitement thermique de tôles d'acier soumises à une déformation longitudinale, comprenant les étapes qui consistent:
à faire passer la tôle le long d'un chemin de cintrage alterné, à une température supérieure à la température critique de l'acier, pour déformer longitudinalement la tôle au-delà de sa limite élastique à ladite température au-dessus de ladite température critique afin d'établir une uniformité substantielle de longueur longitudinale sur toute ladite tôle, supprimant ainsi ladite déformation longitudinale; et
à faire passer la tôle le long d'un bain de trempe tout en refroidissant rapidement et uniformément la tôle d'au-dessus de la température critique jusqu'àu-dessus de sa température de martensite, en même temps que la tôle est retenue longitudinalement et latéralement de façon incrémentielle pour conserver ainsi l'uniformité de la longueur longitudinale.

9. Procédé selon la revendication 8, dans lequel ladite température est d'environ 1650°F (898,9°C) ou plus.

10. Procédé selon la revendication 9, dans lequel la tôle sort dudit cintrage alterné sans chute notable de température et à une température supérieure à environ 1650°F (898,9°C) ou plus.

11. Procédé selon la revendication 10, dans lequel ledit chemin de cintrage alterné présente une courbure qui décroît progressivement afin de travailler à chaud la tôle et d'y égaliser les contraintes internes après l'établissement de ladite uniformité sensible de la longueur longitudinale.

12. Procédé selon la revendication 11, dans lequel la tôle passe le long dudit chemin de cintrage alterné sans être soumise à une tension longitudinale.

13. Procédé selon la revendication 8, dans lequel la tôle est soumise à une contrainte longitudinale dans ledit chemin de cintrage alterné, dans la gemme de 2000 à 3000 psi (137,9-206,8 bars).

14. Procédé selon la revendication 13, comprenant en outre l'étape qui consiste à maintenir la tôle dans un four d'austénitisation à une température supérieure à ladite température critique et à faire passer immédiatement la tôle dans ledit chemin de cintrage alterné sans chute notable de température.

15. Procédé selon la revendication 14, dans lequel on fait passer ladite tôle le long desdits chemins à une vitesse dans la gamme de 20 à 200 feet par minute.

16. Procédé selon la revendication 8, dans lequel les contraintes engendrées dans la tôle après la trempe sont égalisées suffisamment pour empêcher une déformation longitudinale ultérieure lors d'une opération de revenu.

17. Procédé de dressage de tôles d'acier soumises à des variations transversales de longueur longitudinale, comprenant l'étape qui consiste:
à soumettre à des flexions progressives et alternées la tôle à une température au-dessus de la température d'austénite de l'acier, sous une charge comprise dans la gamme d'environ 2000 à 3000 psi (137,9-206,8 bars), suffisante pour éliminer sensiblement les variations transversales de longueur longitudinale.

18. Procédé selon la revendication 17, consistant à atténuer progressivement la flexion de la tôle pour favoriser une égalisation des contraintes dans la tôle.
